

# United States Patent [19]

Anderson, Jr. et al.

[11] 3,753,699

[45] Aug. 21, 1973

[54] **REFRACTORY METAL ALLOYS FOR USE IN OXIDATION ENVIRONMENTS**

[75] Inventors: Wallace T. Anderson, Jr., Huntington Beach; Ralph A. Mendelson, Westminster, both of Calif.

[73] Assignee: TRW Inc., Redondo Beach, Calif.

[22] Filed: Dec. 30, 1971

[21] Appl. No.: 214,351

[52] U.S. Cl. .... 75/174

[51] Int. Cl. .... C22c 27/00

[58] Field of Search..... 75/134, 174, 175.5

[56] **References Cited**

UNITED STATES PATENTS

3,028,236 4/1962 Wlodek et al. .... 75/174  
3,317,314 5/1967 Wlodek et al. .... 75/174

2,940,845 6/1960 Jaffee et al. .... 75/175.5 X  
2,822,268 2/1958 Hix .... 75/174

Primary Examiner—Charles N. Lovell

Attorney—Daniel T. Anderson et al.

[57] **ABSTRACT**

A refractory metal alloy comprising principally columbium and titanium with lesser amounts of hafnium, vanadium, tungsten, aluminum, and molybdenum provides excellent resistance to air oxidation at high temperature.

The preferred composition range is as follows:

Columbium 48–54 percent; Titanium 23–25 percent; Hafnium 9.75–17.5 percent; Vanadium 2–8.75 percent; Tungsten 2.25–2.75 percent; Aluminum 1.8 percent; and Molybdenum 0.7 percent; all parts by weight.

2 Claims, 2 Drawing Figures



PATENTED AUG 21 1973

3,753,699

SHEET 1 OF 2



Fig. 1

PATENTED AUG 21 1973

3,753,699

SHEET 2 OF 2



Fig. 2

## REFRACTORY METAL ALLOYS FOR USE IN OXIDATION ENVIRONMENTS

### BACKGROUND OF THE INVENTION

This invention relates to new and improved refractory metal alloys. More specifically, this invention relates to refractory metal alloys having columbium and titanium as the principal alloy ingredients; hafnium, vanadium, tungsten, aluminum, and molybdenum are minor constituents.

Refractory alloys have been employed as castings, forgings, etc., at high temperatures.

Typical examples of refractory alloys are found in U.S. Pat. Nos. 3,086,859; 2,940,845; 2,991,197; 2,880,088; 2,819,960; 2,754,204; and 3,368,881.

However, their use at high temperature in an oxidizing environment is limited since the amount of oxidation continues with increasing time. Eventually, this results in failure of the alloy as it becomes converted into an oxide.

It is, therefore, an object of the present invention to provide a refractory alloy which may be employed as castings, forgings, etc., in a high temperature, oxidizing environment such as air.

Other objects will be disclosed from the description and graph to follow.

According to the invention, the broad range of the components in the refractory alloy is as follows:

Columbium 48-54 percent; Titanium 23-25 percent; Vanadium 2-8.75 percent; Hafnium 9.75-17.5 percent; Tungsten 2.25-2.75 percent; Aluminum 1.8 percent; and Molybdenum 0.7 percent; all parts by weight percent.

A narrower range of components is as follows:

Columbium 49.5-52.5 percent; Titanium 23-25 percent; Hafnium 10-16.5 percent; Vanadium 2.25-8.5 percent; Tungsten 2.5 percent; Aluminum 1.8 percent; and Molybdenum 0.7 percent; all parts by weight percent.

Specific alloy compositions of this invention are:

| Composition | Columbium | Titanium | Hafnium | Vanadium | Tungsten | Aluminum | Molybdenum |
|-------------|-----------|----------|---------|----------|----------|----------|------------|
| 1.....      | 52.5      | 24.0     | 10.2    | 8.3      | 2.5      | 1.8      | 0.7        |
| 2.....      | 52.5      | 24.0     | 13.2    | 5.3      | 2.5      | 1.8      | 0.7        |
| 3.....      | 52.5      | 24.0     | 16.2    | 2.8      | 2.5      | 1.8      | 0.7        |
| 4.....      | 49.5      | 24.0     | 16.2    | 5.3      | 2.5      | 1.8      | 0.7        |

The oxidation resistance of the present alloys was tested by exposure to air at temperatures between 1,100° C and 1,300° C. The weight gain of the alloys, which is considered to indicate the extent of oxidation, was measured as a function of the exposure time.

In the drawings, FIGS. 1 and 2 are graphs showing

the relationship between exposure times and weight gain (due to oxidation) of the alloy compositions at various oxidation temperatures in air.

FIG. 1 shows a comparison of the oxidation resistance in air of composition 4 with that of a typical prior art refractory metal alloy having the composition 45 at. % Nb; 50 at. % Zr; 5 at. % Ti. It is noted that the curve of composition 4 at 1,300° C is well below that of the prior art alloy when exposed to air at 1,200° C; this represents a significant improvement in oxidation resistance.

In FIG. 2, it will be observed that composition 2 performs about as well at 1,300° C as the prior art alloy does at 1,200° C. Also, at 1,300° C, composition 3 performs significantly better than does the prior art alloy at 1,200° C.

It will also be observed in FIG. 2 that small changes in the alloy composition can be critical to oxidation resistance. For example, decreasing the concentration of columbium (from 49.5 to 46.5 percent) while increasing the vanadium content (from 5.3 to 8.3 percent) results in an alloy having poor oxidation resistance.

The melting point of the present alloy was found to be in excess of 1,700° C; this is at least comparable to refractory metal alloys of the prior art.

Hence, the alloy compositions of this invention are markedly superior to prior art alloys in terms of resistance to air oxidation at high temperature. This factor along with their high melting point renders them well suited for use at high temperatures in air as forgings, castings, etc.

We claim:

1. A refractory alloy consisting of:

Columbium 48-54 percent; Titanium 23-25 percent; Hafnium 9.75-17.5 percent; Vanadium 2-8.75 percent; Tungsten 2.25-2.75 percent; Aluminum 1.8 percent; and Molybdenum 0.7 percent; all parts by weight.

2. A refractory alloy consisting of:

Columbium 49.5-52.5 percent; Titanium 23-25 percent; Hafnium 10-16.5 percent; Vanadium 2.25-8.5 percent; Tungsten 2.5 percent; Aluminum 1.8 percent; and Molybdenum 0.7 percent; all parts by weight.

\* \* \* \* \*